

Jan. 4, 1955

L. GODOWSKY

2,698,794

MIXED PACKET PHOTOGRAPHIC EMULSIONS

Filed April 15, 1950



LEOPOLD GODOWSKY  
INVENTOR

BY Daniel J. Mayne  
R. Frank Smith  
ATTORNEYS

1

2,698,794

## MIXED PACKET PHOTOGRAPHIC EMULSIONS

Leopold Godowsky, Westport, Conn., assignor to Eastman Kodak Company, Rochester, N. Y., a corporation of New Jersey

Application April 15, 1950, Serial No. 156,066

11 Claims. (Cl. 95-2)

This invention relates to color photography and particularly to mixed packet photographic emulsions.

There have been many prior suggestions of mixed grain photographic emulsions, that is, photographic systems in which differently sensitized silver halide grains are incorporated in a single photographic emulsion layer and used to produce differently colored photographic images in the layer. Mixed grain systems have a number of advantages, chief among which is the simplicity of coating a single emulsion layer rather than several layers. Other advantages are the improved definition obtained by having the differently sensitized particles juxtaposed in a single layer, and the simplification of processing which is generally obtained.

Prior mixed grain photographic methods have not been successful either because it was impossible to secure color separation with them, that is, effectively to prevent color formation around unexposed silver halide grains, or because the colored particles formed in the process were too grainy.

It is therefore an object of the present invention to provide a method and sensitive material for mixed packet color photography according to which difficulties in the prior art are overcome and a practical result is achieved. By "mixed packet" I mean a process or an emulsion in which differently color-sensitive silver halide grains having color-formers associated therewith are incorporated in a single photographic layer for the purpose of producing differently colored photographic images in that layer by a single exposure.

These objects are accomplished by first dispersing a color-forming compound in a peptized silver halide emulsion, preferably a gelatino-silver halide emulsion. The emulsion may contain the normal amount of gelatin, or a lower amount than usual may be present. For example, the gelatin content may be from 4 to 200 grams or more per 100 grams of silver halide. The emulsion containing the coupler dispersion is then mixed with a suitable water-dispersible polymer which does not react with gelatin, and to the mixture there is added a solution of a polymeric packet-forming component. Two or more of the resulting packet dispersions which contain silver halide sensitized to different spectral regions, are then mixed with additional gelatin or another water-soluble polymer to form the mixed packet emulsion, preferably by adding the gelatin or polymer to each packet dispersion separately before mixing them.

The accompanying drawing is a flow sheet illustrating the steps in my process.

My invention involves the use of a silver halide emulsion containing a non-diffusing color-forming compound or coupler which is reactive with the oxidation product of a primary aromatic amino developing agent to form a dye image. These couplers are preferably incorporated in the emulsion as described in Jelley and Vittum U. S. Patent 2,322,027, but may be directly dispersed in the

5

10

The following couplers are suitable for use according to my invention:

## CYAN COUPLERS



20

25



30

35



40



45



50



55



60



65





1-(p-[p'-tert.-butylphenoxy]-phenyl)-3-(p-[a-(p'-tert.-butylphenoxy)-propionylamino]-benzoylamino-5-pyrazolone)



1-(p-[p'-tert.-butylphenoxy]-phenyl)-3-(m-[p-toluenesulfonyl-amino]-benzoylamino-5-pyrazolone)

## YELLOW COUPLERS



N-(p-benzoylacetaminobenzenesulphonyl)-N-(n-amylo-tert.-amylaniline)



N-(p-benzoylacetaminobenzenesulphonyl)-N-(gamma-phenylpropyl)-aniline



N-(p-benzoylacetaminobenzenesulphonyl)-N-benzyl-p-toluidine



N-(p-benzoylacetaminobenzenesulphonyl)-N-(gamma-phenylpropyl)-p-tert.-amylaniline



N-(p-benzoylacetaminobenzenesulphonyl)-N-(gamma-phenylpropyl)-o-, m-, or p-toluidine

After making the dispersion of coupler in gelatin-silver halide emulsion, the dispersion is added to a water solution of a water-soluble polymer or water-soluble salt of a polymeric material containing salt-forming acid groups, such as the copolymer of methacrylic acid and methyl-alpha-methacrylate (Minsk, Weyer and McDowell U. S. Patent 2,391,181) algin (alkali metal salt of polymeric d-mannuronic acid), carboxy methyl cellulose (Collins, Freeman and Anthonisen U. S. Patent 2,278,612), and cellulose sulfate (Belgian Patent 448,249). The water-soluble polymer is mixed with the gelatin of the dispersion and acts as a modifying agent, so that small packets, each containing appropriately sensitized silver halide and color-forming coupler, can be formed.

To the mixture of dispersion and water-soluble polymer or salt, mentioned above, there is then added, preferably with stirring, an aqueous solution of a polymeric packet-forming component or gelatin reactant, or vice versa. The polymeric, packet-forming component consists of a polymeric carbon chain having recurring phenyl groups and carboxyl groups, and preferably also carboxylic acid amide groups or imide groups or both and is used as the water-soluble salt, such as the ammonium, sodium, potassium or lithium salt. The polymeric packet-forming component is preferably an interpolymer of styrene and an alpha,beta-unsaturated carboxylic acid, part of whose carboxyl groups may have been converted to

amide or imide derivatives or both, such as interpolymers of styrene-maleic acid, styrene-acrylic acid, styrene-methacrylic acid or styrene-itaconic acid.

The mixture of coupler-silver halide dispersion, water-soluble polymer and polymeric packet-forming component now consists of particles or packets of gelatin, associated with polymeric packet-forming component containing silver halide and coupler, the packets being dispersed in an aqueous medium containing additional gelatin or another film-forming water-soluble polymer. This is finally mixed with at least one other similarly made packet dispersion containing differently-sensitized silver halide and a different coupler to form the finished mixed grain emulsion. The finished emulsion is then ready for coating on a suitable support, such as glass, cellulose ester, or paper.

In the preparation of the system described above, that is, gelatin, water-soluble polymer, and packet-forming component, the ingredients must be present in a fairly definite ratio. If the gelatin is present in approximately 0.7% aqueous solution (an appropriate concentration for making an emulsion), then the water-soluble polymer should be present in an amount from about 1 to 2 times that of the gelatin, and the packet-forming component should be present in an amount from 0.01 to 0.5 times that of the gelatin. Within these ranges the three-component systems exhibit a definite degree of optical turbidity. If this turbidity is measured in optical density per cm. of mixture at 30° C., using orange-colored light, of about 5800 A. U., the optical density is greater 0.05, and is generally of the order of 0.1.

Suitable polymers of styrene with maleic acid or its derivatives are represented by the following formula:



Suitable polymers of styrene with acrylic acid or its derivatives may be represented by the following formula:



In each formula—

Y=OH

NH<sub>2</sub>

NHR'

NR'2

R=hydrogen

CH<sub>3</sub>

C<sub>2</sub>H<sub>5</sub>

R'=alkyl of less than six carbon atoms or aryl

Z=NH

NR'

OH

groups on each carbon atom to which Z is attached.

n=the number of units in the polymer chain.

It will be understood that the above structural formulas

are illustrative only, and are not limiting as to ratios and unit arrangements of constituents.

The polymeric packet-forming components of the first structural formula above may be prepared by forming an interpolymer of styrene and maleic anhydride, and then treating the polymer with ammonia, a primary or secondary amine, or water, as indicated by the following formula using ammonia:



Formation of these polymers is described in Condo, Krister and Lundquist U. S. Patent 2,286,062 and McDowell and Kenyon U. S. Patent 2,313,565.

Interpolymers of styrene and acrylic anhydride or  $\alpha$ -methacrylic anhydride may be used instead of the interpolymer of styrene and maleic anhydride, as indicated by the following formula using ammonia:



Imide groups along the polymer chain may result from the interaction of adjacent amide groups or an amide and a carboxyl group.

These polymers may also be prepared by direct polymerization, e. g., styrene, acrylamide or N-substituted acrylamide, acrylic acid; or styrene, maleamic acid or N-substituted maleamic acid.

In order to ascertain the packet-forming components which are suitable for use in my process, the following test may be made:

A solution or dispersion of the polymeric compound to be tested, gelatin, and the sodium salt of methylmethacrylate-methacrylic acid polymer is made up in water so that the final concentrations are gelatin, 0.7%; methylmethacrylate-methacrylic acid salt, 1.67 times the amount of gelatin; and polymeric compound, 0.1 to 0.5 times the amount of gelatin. The gelatin is a deashed calfskin gelatin having an isoelectric point of approximately 4.8. The polymeric compound is added as an approximately 2% solution in ammonium hydroxide of pH 7.5. When vigorously stirred, this mixture is characterized by its ability to scatter or diffuse light transmitted through it. With polymeric compounds suitable for my process, the mixture must exhibit an optical density of at least 0.05 per centimeter of mixture, when measured at 30° C. with orange-colored light of approximately 5800 Angstrom units wave length.

The packet-forming components were prepared as follows:

*Example 1.—Styrene-maleic anhydride interpolymer*

Into a 12-liter all glass reflux outfit equipped for anhydrous conditions the following were measured:

234 gm. distilled styrene  
220.5 gm. maleic anhydride  
3188 ml. dry benzene  
4.25 gm. benzoyl peroxide

The reaction mixture was heated on a steam bath for a total of two hours although the major portion of the reaction was completed in less than twenty minutes after the steam had been turned on. When the reaction mixture had cooled to room temperature, the solids were separated by filtration, washed with dry benzene and put to dry in a vacuum oven at 60° C.

*Example 2.—Polystyrene-maleamic acid polymer*

50 gm. of polystyrenemaleic anhydride were added gradually to 250 ml. of 28% ammonium hydroxide in a

500 ml. Erlenmeyer flask with stirring from a mixer to form a slurry. After stirring for eighteen hours at room temperature a viscous, clear colorless dope was obtained.

300 gm. of this dope was diluted to approximately 2% solids with water and 48% hydrobromic acid was added to it until it was just acid to Congo red. The solid that was formed was separated by filtration, and leached with absolute alcohol until the wash solutions were bromide free. The solids were put to dry in an oven at 60° C.

10 20 gm. of the solid were doped to form a 5% dope by weight in water made alkaline with 13 ml. of 20% sodium hydroxide. pH=8.63.

*Example 3.—Polystyrene-maleamic acid ammonium salt*

15 The following reagents were put to reflux in an all glass reflux outfit equipped with a mechanical stirrer. Conditions were maintained anhydrous by calcium chloride tubes on all openings to the atmosphere.

20 49 gm. maleic anhydride (Eastman white label)  
52 gm. distilled styrene  
1500 ml. dry toluene  
2.0 gm. benzoyl peroxide

The reaction mixture was heated for 2½ hours on a steam bath without stirring and then allowed to cool to room temperature. A small sample of the solids was withdrawn, washed with fresh benzene, and put to dry for analysis and viscosity purposes.

The stirrer was turned on and dry ammonia was bubbled into the reaction mixture continuously for 3½ hours. During this time the temperature within the reaction mixture rose from a starting temperature of 23° C. to 45° C. and then returned to 23° C. The solids were filtered off on a Büchner funnel, washed with toluene, and put to dry in a vacuum oven at 60° C. over night.

The residual toluene was then extracted with absolute alcohol by stirring the product with 2-3 l. portions of absolute ethyl alcohol and filtering onto a Büchner funnel. The product was then dried as above.

40 Forty grams of the polymer were gradually added to 200 ml. of water in an Erlenmeyer flask with mechanical stirring. The solution was kept slightly alkaline by the portion-wise addition of 28% NH<sub>4</sub>OH. The pH was never allowed to exceed eight. A clear colorless dope

45 was obtained which was then adjusted to 15% solids by weight by the addition of distilled water. The pH of this solution was 6.38.

*Example 4.—Ammonium salt of styrene-maleic acid interpolymer*

50 10 gm. of a styrene-maleic anhydride interpolymer were heated with 200 ml. of distilled water on a steam bath for 6 hours and then left at room temperature for 65 hours. After this period of hydrolysis, 28% NH<sub>4</sub>OH was added to the mixture portion-wise while it was mechanically stirred, using no more ammonium hydroxide than was necessary to effect solution. The solution was then diluted to 400 g. total weight with distilled water. The pH of the solution was 6.34.

*Example 5.—Sodium salt of styrene-maleic acid interpolymer*

The procedure was similar to the above example except that 10% sodium hydroxide was used to effect solution

65 of the hydrolyzed styrene-maleic anhydride interpolymer. The pH of the final solution was 8.16.

*Example 6.—Styrene-acrylic anhydride copolymer*

The following were heated in an all glass reflux outfit

70 on a steam bath under anhydrous conditions for 24 hours:

42 gm. distilled acrylic anhydride  
35 gm. distilled styrene  
500 ml. dry 1,4-dioxane  
0.8 ml. 30% H<sub>2</sub>O<sub>2</sub>

75 The reaction mixture was shaken frequently. During the first hour the mixture began to become cloudy; shortly after this period, the mixture became very cloudy and set to a gel. After cooling to room temperature, the solids were broken up, separated by filtration and washed with dry dioxane. The polymer was dried in vacuum desiccator under constant water pump vacuum, with a calcium chloride tube in the vacuum line.

Preparation of the styrene-acrylic acid-acrylamide polymer was carried out similar to the preparation of the

7  
polystyrene-maleamic acid polymer in aqueous ammonium hydroxide, only using the above intermediate.

*Example 7.—Methacrylic anhydride-styrene interpolymer*

The following were mixed in an all glass reflux apparatus and refluxed on a steam bath for 16 hours protected from moisture by a calcium chloride tube.

61.6 gm. distilled methacrylic anhydride  
41.6 gm. distilled styrene  
1.0 ml. 30%  $H_2O_2$   
600 ml. dry 1,4 dioxane

The solution gelled after the first hour and half of heating. When the reaction mixture had cooled to room temperature after the 16 hour heating period, the gel was manually broken up and washed with dry 1,4-dioxane in a Büchner funnel. The product was dried.

The preparation of the styrene methacrylic acid, methacrylamide polymer was carried out exactly similar to the preparation of the polystyrene-maleamic acid polymer in ammonium hydroxide.

*Example 8.—Maleic anhydride: styrene: vinyl acetate interpolymer*

The following were put in a resin reaction flask equipped with a reflux condenser and mechanical stirrer:

196 grams distilled maleic anhydride  
145 grams distilled styrene  
51.6 grams distilled vinyl acetate  
1 liter dry benzene  
2.0 ml. 30 per cent hydrogen peroxide

The reaction mixture was protected from moisture by calcium chloride tubes in openings to the atmosphere. Slow stirring was maintained and the flask was kept in a constant temperature bath at 60° C. for 24 hours. At the end of this time, the precipitate was removed from the reaction flask, washed with dry benzene, and put to dry in a vacuum desiccator under constant water pump vacuum.

*Example 9.—Maleamic acid:styrene:vinyl acetate interpolymer*

Fifty grams of the styrene-vinyl acetate-maleic anhydride interpolymer (Example 8) were added to 350 cc. of 28 per cent ammonium hydroxide with stirring. The mixture was stirred for 16 hours, during which time solution occurred and a viscous dope was obtained. This was diluted to 1220 grams with distilled water, making a 5 per cent solution. Two hundred grams of the above dope were diluted to 750 cc. with distilled water and then made acid to Congo red with hydrobromic acid. The precipitate was filtered and then extracted with absolute ethyl alcohol until bromide-free. The product was then dried in vacuum. The yield was 7 grams. This was dispersed by stirring in water containing ammonium hydroxide.

*Example 10.—Maleic anhydride:styrene:butyl acrylate interpolymer*

The following were put in an all-glass reflux outfit equipped for anhydrous conditions on a steam bath to reflux for 2 hours:

36.4 grams distilled styrene  
49.0 grams maleic anhydride  
19.2 grams distilled butyl acrylate  
1.0 gram benzoyl peroxide  
750 ml. dry benzene

When the reaction was completed, the reaction mixture was cooled to room temperature. The resulting precipitate was isolated by filtration on a Büchner funnel, washed with dry benzene, and put to dry in a vacuum desiccator under constant water pump vacuum. The yield was 76.0 grams. Inherent viscosity, 0.66. (See Cragg, J. Colloid Science, vol. 1, page 261, 1946, for description of inherent viscosity.)

*Example 11.—Maleamic acid:butyl acrylate:styrene interpolymer*

Forty grams of the interpolymer of styrene-butyl acrylate and maleic anhydride interpolymer (Example 10) were added with stirring to 200 cc. of 28 per cent ammonium hydroxide kept chilled in an ice bath. In 20 minutes a viscous dope was obtained and 100 cc. of water

were added. The reaction mixture was stirred for 2 hours with continued chilling. The smooth dope obtained was diluted to 1600 grams and then the pH was adjusted to 7.9 with 6-N sulfuric acid. Four hundred grams of this dope were diluted to 800 cc. with distilled water and made acid to Congo red with 20 per cent hydrobromic acid. The precipitate was filtered and extracted with absolute ethyl alcohol until bromide-free. The product was then dried in vacuum. The yield was 11.5 grams. This was dispersed as described in Example 9.

*Example 12.—Styrene N-butyl maleamic acid interpolymer*

Forty and four-tenths grams of styrene-maleic anhydride interpolymer (inherent viscosity, 0.68) were dispersed with shaking in 404 cc. of dry methyl ethyl ketone. To the dope was added with stirring a solution of 14.6 grams of *N*-butylamine in 404 cc. of dry methyl ethyl ketone. There was instant precipitation. The mixture was well shaken and left at room temperature for 17 hours. The polymer had then precipitated as a cake which was broken up and to the mixture was added 50 cc. of 28 per cent ammonium hydroxide. The reaction mixture was then allowed to stand for 5 hours. The precipitate was then filtered, reextracted with methyl ethyl ketone and dried in vacuum. The yield was 64 grams.

Forty grams of this polymer were dispersed in 1000 cc. of distilled water to which had been added 10 cc. of 28 per cent ammonium hydroxide. Solution occurred. The dope was diluted to 1600 grams, making a concentration of 2.5 per cent in solids. The pH was 9.0.

To isolate the acid form of the polymer, 400 grams of this dope diluted with an equal part of water were made acid to Congo red with 20 per cent hydrobromic acid. The precipitate was filtered, extracted with water until bromide-free, and dried in vacuum. The yield was 7 grams. When a portion of this precipitate was redispersed in water by the addition of ammonium hydroxide, it was found to yield packets.

*Example 13.—Polystyrene:N-diethyl maleic acid*

Thirty grams of (1:1) polystyrene:maleic anhydride dried polymer were added slowly to 200 ml. of diethylamine and 200 ml. of water with constant stirring by a mixer. After 7 hours' stirring at room temperature, a syrupy clear amber dope was obtained. The dope was thinned to approximately 3 per cent solids with water and then made just acid to Congo red with 48 per cent hydrobromic acid. The resulting precipitate was isolated by filtration and washed with water until bromide-free. The product was then dried in a vacuum desiccator under constant water pump vacuum.

To prepare the ammonium salt of the polystyrene *N*-diethyl maleamic acid, 10 grams of the acid polymer were added to 75 ml. of water with stirring by a mixer. Twenty-eight per cent  $NH_4OH$  was added portionwise to keep the pH at about 8. After 12 hours' stirring a light amber dope was obtained. This dope was filtered and diluted to 6.66 per cent solids, pH 8.33.

*Example 14.—Copolymer of styrene:acrylamide:acrylic acid*

The following were put in an all-glass reflux outfit:

52 grams styrene  
35.5 grams acrylamide  
36 grams acrylic acid  
1.225 grams benzoyl peroxide  
367.5 grams absolute ethyl alcohol

The reaction mixture was heated on a steam bath for 23 hours. A slightly turbid dope was obtained which, upon cooling, deposits polymer. The hot dope was poured into distilled water to precipitate the polymer. The precipitate was washed with distilled water, after which it was dried in an air oven at room temperature. The yield was 73.5 grams, nitrogen content 3.5%. The product dissolved in water at elevated pH.

This material was dispersed in water by the addition of ammonium hydroxide.

80 A two-color emulsion was made as follows:

*Example 15*

Separate red-sensitive and green-sensitive silver bromoiodide emulsions were made containing 33 grams of gelatin per 100 grams of silver halide.

A cyan coupler dispersion was made by dissolving 4.375 grams of the coupler 2-[ $\alpha$ -(2,4-di-tert.-amylphenoxy)-n-butyrylaminol-4,6-dichloro-5-methyl phenol and 0.27 gram of diethyl hydroquinone in 5 cc. of n-butylphthalate at 150° C. adding the solution to 5 cc. of a 5% solution of Alkanol B dispersing agent in 25 cc. of 10% gelatin solution, and dispersing it therein.

A magenta coupler dispersion was made by dissolving 2.75 grams of the coupler 1-(p'-tert.-butyl-phenoxy-phenyl) - 3 - [m.-(p-tert.-amylphenoxy)benzoylaminol-5-pyrazolone and 0.21 gram of diethyl hydroquinone in 7.9 cc. of n-butylphthalate at 165° C., adding the solution to 5 cc. of a 5% solution of Alkanol B in 25 cc. of 10% gelatin solution, and dispersing it therein.

Six grams of the red-sensitive emulsion containing 0.4 gram of silver halide and 0.13 gram of gelatin were added to 8 grams of the cyan coupler dispersion and mixed with a fast stirrer for 10 minutes. Twelve cc. of a 10% solution of a copolymer of methacrylic acid and methyl- $\alpha$ -methacrylate (sodium salt) were mixed with 100 cc. of distilled water. The emulsion-coupler dispersion was added to the copolymer solution, and this was stirred for 10 minutes more. To this mixture there were added 4 cc. of a 0.5% solution of the ammonium salt of styrene-maleamic acid polymer, and the whole dispersion was stirred at 42° C. for one hour. Then 50 cc. of an 18% solution of gelatin were added and mixed.

A similar dispersion was made using 6 grams of the green-sensitive emulsion containing 0.4 gram of silver halide and 0.13 gram of gelatin, and 8 grams of the magenta coupler dispersion instead of the red-sensitive emulsion and cyan coupler.

The two final dispersions were mixed together and coated, and after exposure and development in a p-phenylene-diamine type color developer, gave satisfactory cyan and magenta images in the portions exposed to red and green light, respectively.

A three-color emulsion was made as follows:

*Example 16*

A yellow-forming coupler dispersion was made by first dissolving 5 grams of the coupler N-(p-benzoyl acetamino benzene sulfonyl)-N-( $\gamma$ -phenylpropyl)-p-toluidine and 0.21 gram of diethyl hydroquinone in 8 grams of dibutyl phthalate at 140-150° C. This solution was added to 25 grams of 10% gelatin solution containing 5 cc. of a 5% solution of Alkanol B dispersing agent and the mixture stirred for five minutes. Six grams of a concentrated gelatino-silver bromoiodide emulsion containing 2.04 grams of silver halide and 0.095 gram of gelatin were then added to 8 grams of the coupler dispersion and the mixture stirred for 15 minutes at 40° C. The mixture was then added to 12 cc. of a 10% solution of a copolymer of methacrylic acid and methyl- $\alpha$ -methacrylate (sodium salt) in 100 cc. of water which had been stirred at 40° C. for 10 minutes. To this mixture there were added 5 cc. of a 0.5% solution of the ammonium salt of styrene-maleamic acid polymer and the whole dispersion was stirred for 12 minutes more. The mixture was then added to 50 grams of an 18% gelatin solution.

A cyan-forming coupler dispersion was made by dissolving 3.5 grams of the coupler 2-[ $\alpha$ -(2',4'-tert.-amylphenoxy)-n-butyryl aminol, 4,6-dichloro-5-methylphenol and 0.21 gram of diethyl hydroquinone in 8 grams of dibutyl phthalate at 140-150° C. This solution was added to 25 grams of a 10% solution of gelatin containing 5 cc. of a 5% solution of Alkanol B and was stirred for five minutes. Eight grams of this coupler dispersion were added to 5.25 grams of a red-sensitive 95 mole per cent chloride, silver chlorobromide emulsion containing 1.24 grams of silver halide and 0.43 gram of gelatin, prepared by adding 5 milligrams of the red sensitizer, 5[4-(3-ethyl-2-(3)-benzothiazolylidene)-2-butenyldiene]-3-n-heptyl-1-phenyl-2-thiohydantoin (U. S. Patent 2,282,116) in 8 cc. of acetone to 66 grams of the emulsion, and the mixture was stirred for 15 minutes at 40° C. The mixture was then added to 12 grams of a 10% solution of a copolymer of methacrylic acid and methyl- $\alpha$ -methacrylate (sodium salt) in 100 cc. of water which had been stirred for 15 minutes at 40° C. The mixture was stirred for 10 minutes at 40° C. and to it was added 5 cc. of a 0.5% solution of the ammonium salt of styrene-maleamic acid polymer and the mixture was stirred for 10 minutes more.

It was then added to 50 cc. of an 18% gelatin solution and mixed.

A magenta-forming coupler dispersion was made by first dissolving 2.75 grams of the coupler, 1-[p-(p'-tert.-butyl-phenoxy)-phenyl] - 3 - [m-(p-tert.-amylphenoxy)benzoylaminol-5-pyrazolone and 0.21 gram of diethyl hydroquinone in eight grams of dibutyl phthalate at 170-180° C. This solution was added to 25 cc. of a 10% gelatin solution containing 5 cc. of a 5% solution of Alkanol B and was stirred for five minutes. Eight grams of this dispersion were added to 5.25 grams of a green-sensitive 95 mole per cent chloride, silver chlorobromide emulsion containing 1.24 grams of silver halide and 0.43 gram of gelatin made by sensitizing 66 grams of the emulsion with 7½ milligrams of the green-sensitizer 5-[1-ethyl-2-(3)- $\alpha$ -naphthoxazolylidene]-ethylidene]-3-n-heptyl-1-phenyl-2-thiohydantoin (U. S. Patent 2,282,116) in 10 cc. of methanol. This mixture was then added to a solution of a copolymer of methacrylic acid and methyl- $\alpha$ -methacrylate (sodium salt) and a solution of the ammonium salt of styrene-maleamic acid polymer in the same way as the red-sensitive emulsion described above.

To produce a three-color coating, 60 grams of each of the blue-sensitive, green-sensitive and red-sensitive components were mixed with stirring. The mixture was then coated in the usual manner on a paper support and dried. After exposure and development in a developing solution containing 2-amino-5-diethyl amino toluene hydrochloride as the developing agent, colored images complementary to the color of the exposing light were formed in the emulsion.

I claim:

1. A light-sensitive mixed packet photographic emulsion comprising packets or discrete particles of gelatin reacted with a water-soluble salt of an interpolymer of styrene and an  $\alpha$ , $\beta$ -unsaturated carboxylic acid, said particles or packets containing a non-diffusing color-forming compound capable of reacting with the oxidation product of a primary aromatic amino developing agent on photographic development, and silver halide sensitive to at least one region but less than all regions of the visible spectrum, and at least one separate set of packets or discrete particles of gelatin reacted with said interpolymer containing a non-diffusing color-forming compound different from said first mentioned color-forming compound and silver halide sensitive to a region of the visible spectrum different from that to which said first mentioned silver halide is sensitive, the sensitive and color-forming ingredients being within the respective packets or discrete particles and all of said packets or discrete particles being dispersed in gelatin having mixed therewith a water-soluble salt of a polymer selected from the class consisting of methylmethacrylate-methacrylic acid copolymer, algin, carboxy methyl cellulose and cellulose sulfate.

2. A light-sensitive mixed packet photographic emulsion comprising packets or discrete particles of gelatin reacted with the ammonium salt of a styrene-maleamic acid polymer, said particles or packets containing a non-diffusing color-forming compound capable of reacting with the oxidation product of a primary aromatic amino developing agent on photographic development, and silver halide sensitive to at least one region but less than all regions of the visible spectrum and at least one separate set of packets or discrete particles of gelatin reacted with said polymer, containing a non-diffusing color-forming compound different from said first mentioned color-forming compound and silver halide sensitive to a region of the visible spectrum different from that to which said first mentioned silver halide is sensitive, the sensitive and color-forming ingredients being within the respective packets or discrete particles and all of said packets being dispersed in gelatin having mixed therewith the sodium salt of methylmethacrylate methacrylic acid copolymer.

3. A photographic element comprising a support having thereon a single light-sensitive water-permeable colloid layer containing (1) packets or discrete particles of gelatin reacted with the ammonium salt of a styrene-maleamic acid polymer, said particles or packets containing a non-diffusing yellow-forming coupler and blue-sensitive silver halide, (2) packets or discrete particles of gelatin reacted with the ammonium salt of a styrene-maleamic acid polymer, said particles or packets containing a non-diffusing magenta-forming coupler and green-sensitive silver halide, and (3) packets or discrete particles of gelatin reacted

with the ammonium salt of a styrene-maleamic acid polymer, said particles or packets containing a non-diffusing cyan-forming coupler and red-sensitive silver halide, and said colloid layer having mixed therewith the sodium salt of methylmethacrylate-methacrylic acid copolymer.

4. The method of making a mixed packet photographic emulsion which comprises dispersing in a gelatino-silver halide emulsion sensitive to at least one but less than all regions of the visible spectrum, a non-diffusing color-forming compound capable of reacting with the oxidation product of a primary aromatic amino developing agent on photographic development to form a dispersion of the color-forming compound in the emulsion, mixing said dispersion with from about one part to about two parts per part of gelatin in said emulsion, of a water-soluble salt of a polymer selected from the class consisting of methylmethacrylate-methacrylic acid copolymer, algin, carboxy methyl cellulose and cellulose sulfate, adding to the mixture of dispersion and polymer slowly and with stirring a solution of a water-soluble salt of an interpolymer of styrene, said interpolymer containing at least a carboxylic acid group of the groups selected from the class consisting of carboxylic acid and carboxylic acid amide groups to form a dispersion of particles of gelatin, water-soluble salt of styrene interpolymer and silver halide, containing the color-forming compound, forming in the same way as said last-mentioned dispersion at least one other dispersion of particles of gelatin, water-soluble salt of styrene interpolymer, different non-diffusing color-forming compound and silver halide sensitive to a region of the visible spectrum different from that to which said first-mentioned silver halide is sensitive, in each of said dispersions said water-soluble polymer being used in an amount from about 1 to about 2 times the amount of gelatin, and said water-soluble salt of styrene interpolymer being used in an amount less than about one-half the amount of gelatin, and mixing said dispersions of particles with a gelatin solution.

5. The method of making a mixed packet photographic emulsion which comprises mixing a non-diffusing color-forming compound capable of reacting with the oxidation product of a primary aromatic amino developing agent on photographic development, with a substantially water-insoluble solvent for said color-forming compound to form a solution of the color-forming compound in the solvent, dispersing the solution in a gelatino-silver halide emulsion sensitive to at least one but less than all regions of the visible spectrum, mixing said dispersion with from about one part to about two parts per part of gelatin in said emulsion, of a water-soluble salt of a polymer selected from the class consisting of methylmethacrylate-methacrylic acid copolymer, algin, carboxy methyl cellulose and cellulose sulfate, adding to the mixture of dispersion and polymer slowly and with stirring a solution of a water-soluble salt of an interpolymer of styrene, said interpolymer containing at least a carboxylic acid group of the groups selected from the class consisting of carboxylic acid and carboxylic acid amide groups to form a dispersion of particles of gelatin, water-soluble salt of styrene interpolymer and silver halide sensitive to a region of the visible spectrum different from that to which said first-mentioned silver halide is sensitive, in each of said dispersions said water-soluble polymer being used in an amount from about 1 to about 2 times the amount of gelatin, and said water-soluble salt of styrene interpolymer being used in an amount less than about one-half the amount of gelatin, and mixing said dispersions of particles with a gelatin solution.

6. A photographic mixed packet dispersion, the continuous phase comprising an aqueous colloidal binder and the disperse phase comprising at least two differently light-sensitive sets of packets or discrete particles, each packet of any one set itself containing dispersed therein silver halide grains sensitized to one of the primary regions of the visible spectrum and also containing dispersed therein a non-diffusing color-forming compound capable of reacting with the oxidation product of a primary aromatic amino developing agent on photographic

development, the particles of any one set being formed when a water-soluble salt of a styrene interpolymer containing carboxylic acid groups is added in the presence of a water-soluble salt of methyl methacrylate-methacrylic acid, to a silver halide dispersion peptized by gelatin, the styrene interpolymer-gelatin combination which forms the continuous phase of the packets being immiscible with said aqueous colloidal binder.

7. The method of making a mixed packet photographic emulsion which comprises mixing a non-diffusing color-forming compound capable of reacting with the oxidation product of a primary aromatic amino developing agent on photographic development, with a substantially water-insoluble solvent for said color-forming compound to form a solution of the color-forming compound in the solvent, dispersing the solution in a gelatino-silver halide emulsion sensitive to at least one region but less than all regions of the visible spectrum, mixing said dispersion with from about 1 part to about 2 parts of the sodium salt of methyl-methacrylate methacrylic acid copolymer, adding to the mixture of dispersion and polymer slowly and with stirring a solution of a polymeric carbon chain compound having recurring phenyl groups, carboxyl groups and amide groups appended thereto to form a dispersion of particles of gelatin, polymeric compound and silver halide containing the color-forming compound, forming in the same way as said last-mentioned dispersion, at least one other dispersion of particles of gelatin, polymeric compound, different non-diffusing color-forming compound and silver halide sensitive to a region of the visible spectrum different from that to which said first-mentioned silver halide is sensitive, in each of said dispersions said copolymer being used in an amount from about 1 to about 2 times the amount of gelatin, and said polymeric compound being used in an amount less than one-half the amount of gelatin, and mixing said dispersions of particles with a gelatin solution.

8. The method of making a mixed packet photographic emulsion which comprises mixing a non-diffusing color-forming compound capable of reacting with the oxidation product of a primary aromatic amino developing agent on photographic development, with a substantially water-insoluble solvent for said color-forming compound to form a solution of the color-forming compound in the solvent, dispersing the solution in a gelatino-silver halide emulsion sensitive to at least one region but less than all regions of the visible spectrum, mixing said dispersion with from about 1 part to about 2 parts of the sodium salt of methyl-methacrylate methacrylic acid copolymer, adding to the mixture of dispersion and polymer slowly and with stirring a solution of styrene interpolymer having carboxyl groups on the polymeric chain, to form a dispersion of particles of gelatin, interpolymer and silver halide containing the color-forming compound, forming in the same way as said last-mentioned dispersion, at least one other dispersion of particles of gelatin, interpolymer, different non-diffusing color-forming compound and silver halide sensitive to a region of the visible spectrum different from that to which said first-mentioned silver halide is sensitive, in each of said dispersions said copolymer being used in an amount from about 1 to about 2 times the amount of gelatin, and said interpolymers being used in an amount less than one-half the amount of gelatin, and mixing said dispersions of particles with a gelatin solution.

9. The method of making a mixed packet photographic emulsion which comprises mixing a non-diffusing color-forming compound capable of reacting with the oxidation product of a primary aromatic amino developing agent on photographic development, with a substantially water-insoluble solvent for said color-forming compound to form a solution of the color-forming compound in the solvent, dispersing the solution in a gelatino-silver halide emulsion sensitive to at least one region but less than all regions of the visible spectrum, mixing said dispersion with from about 1 part to about 2 parts of the sodium salt of methylmethacrylate-methacrylic acid copolymer, adding to the mixture of dispersion and polymer slowly and with stirring a solution of interpolymer of styrene and an  $\alpha,\beta$ -unsaturated carboxylic acid to form a dispersion of particles of gelatin, interpolymer and silver halide containing the color-forming compound, forming in the same way as said last-mentioned disper-

sion, at least one other dispersion of particles of gelatin, interpolymer, different non-diffusing color-forming compound and silver halide sensitive to a region of the visible spectrum different from that to which said first-mentioned silver halide is sensitive, in each of said dispersions said water-soluble polymer being used in an amount from about 1 to about 2 times the amount of gelatin, and said interpolymer being used in an amount less than one-half the amount of gelatin, and mixing said dispersions of particles with a gelatin solution.

10. A light-sensitive mixed packet photographic emulsion comprising packets or discrete particles of gelatin reacted with a water-soluble salt of an interpolymer of styrene, said interpolymer containing at least a carboxylic acid group of the groups selected from the class consisting of carboxylic acid and carboxylic acid amide groups, said particles or packets containing a non-diffusing color-forming compound capable of reacting with the oxidation product of a primary aromatic amino developing agent on photographic development, and silver halide sensitive to at least one region but less than all regions of the visible spectrum, and at least one separate set of packets or discrete particles of gelatin reacted with said interpolymer, containing a non-diffusing color-forming compound different from said first-mentioned color-forming compound and silver halide sensitive to a region of the visible spectrum different from that to which said first-mentioned silver halide is sensitive, the sensitive and color-forming ingredients being within the respective packets or discrete particles and all of said packets or discrete particles being dispersed in gelatin and having mixed therewith the sodium salt of methylmethacrylate-methacrylic acid copolymer.

11. A light-sensitive mixed packet photographic emulsion comprising packets or discrete particles of gelatin reacted with the ammonium salt of styrene-acrylamide-acrylic acid interpolymer, said particles or packets containing a non-diffusing color-forming compound capable of reacting with the oxidation product of a primary aromatic amino developing agent on photographic development, and silver halide sensitive to at least one region but less than all regions of the visible spectrum, and at least one separate set of packets or discrete particles of gelatin reacted with said interpolymer, containing a non-diffusing color-forming compound different from said first-mentioned color-forming compound and silver halide sensitive to a region of the visible spectrum different from that to which said first-mentioned silver halide is sensitive, the sensitive and color-forming ingredients being within the respective packets or discrete particles and all of said packets or discrete particles being dispersed in gelatin and having mixed therewith the sodium salt of 20 methylmethacrylate-methacrylic acid copolymer.

## References Cited in the file of this patent

## UNITED STATES PATENTS

|    |           |               |               |
|----|-----------|---------------|---------------|
| 25 | 1,976,679 | Fikentscher   | Oct. 9, 1934  |
|    | 2,284,877 | Martinez      | June 2, 1942  |
|    | 2,399,084 | Watson        | Apr. 23, 1946 |
|    | 2,490,749 | Fierke et al. | Dec. 6, 1949  |
|    | 2,548,526 | Godowsky      | Apr. 10, 1951 |
| 30 | 2,565,418 | Yackel        | Aug. 21, 1951 |